

## UNITED STATES PATENT OFFICE

2,020,698

PILE FABRIC AND METHOD OF  
TREATING THE SAME

Herbert Platt, Cumberland, Md., assignor to Celanese Corporation of America, a corporation of Delaware

No Drawing. Application October 24, 1933,  
Serial No. 695,003

14 Claims.

(Cl. 26—2)

This invention relates to the production of differential lustre effects and differential pile effects on fabrics having a pile comprising organic esters of cellulose.

5 An object of my invention is to produce differential lustre effects on fabrics having a pile comprising organic ester of cellulose yarn by the local application thereto of a saponifying agent. Other objects of this invention will appear from the following detailed description.

I have found that if a saponifying agent is applied to a fabric having a pile of organic ester of cellulose yarn, such yarn, because of the conversion of the cellulose ester in part or in whole to regenerated cellulose, has imparted thereto different properties, such as different lustre, covering power, dyeing properties, and behavior towards the steps involved in the finishing of velvets. By locally applying a saponifying agent to such fabrics, it is possible to obtain differential effects that are highly ornamental and which cannot be obtained in any other manner.

In accordance with my invention then I produce ornamental effects on a fabric having a pile comprising organic ester of cellulose yarn by locally applying thereto a composition containing a saponifying agent for the cellulose ester.

The fabric to be treated has a pile which comprises yarns of organic esters of cellulose, such as cellulose acetate, cellulose formate, cellulose propionate and cellulose butyrate. The pile may consist wholly of such organic ester of cellulose yarn, or may also comprise yarns of other fibres such as regenerated cellulose, cotton, natural silk.

35 The back of the fabric to be treated may be made of or contain organic ester of cellulose yarn, or may be made in whole or in part of other fibres such as natural silk, regenerated cellulose, cotton, etc.

40 The fabric has locally applied thereto a saponifying agent which comprises an alkali or alkaline salt that saponifies at least partially the cellulose ester. Examples of such alkaline materials are sodium hydroxide, potassium hydroxide, sodium carbonate, etc. The alkaline agent is present in rather concentrated form, in case of sodium hydroxide the amount being 10 to 30% by weight. The saponifying agent is generally applied in the form of a paste containing thickening agents such as gum tragacanth, British gum or other dextrines, water-soluble cellulose ethers, agar agar, starches or the like.

45 In order to obtain better penetration and quicker action of the alkaline material, the saponifying agent may contain a swelling agent for

the cellulose acetate or other organic ester of cellulose, examples of which are pyridine, the thiocyanates of sodium, potassium or ammonium, ethyl alcohol, methyl alcohol, diethylene glycol, etc.

5 The fabric so produced has differential lustre or "shadow print" effects. This differential effect may be enhanced by treating the fabric in various manners.

10 The organic ester of cellulose pile yarns that have not been saponified are more difficult to change from their position after they are once set than are the saponified organic ester of cellulose yarns. Therefore it is possible to obtain a differential lay between the saponified and unsaponified organic ester of cellulose pile yarn. Thus the fabric, after the application of the saponifying agent, may be washed, finished and dried with the pile erect, after which the fabric 15 may be run through water and brushed across the piece to lay the pile towards the selvage and is then dried. This causes the saponified pile 20 yarn to lie flat while the unsaponified yarn remains substantially erect. Upon subsequent steaming and cross-brushing the fabric in the 25 opposite direction, any unsaponified yarn which may have been slightly bent from the vertical by the previous brushing toward the selvage is caused to stand erect without disturbing the position of the laid or crushed saponified organic 30 ester of cellulose pile yarn.

35 The saponified organic ester of cellulose yarn has an affinity for cotton colors. Therefore by treating the fabric after local application of the saponifying agent with a dye-bath containing both cotton dyes and dyes having an affinity for organic ester of cellulose material, differential color effects may be produced. If the back is made of natural silk, three color effects may be obtained by using a dye having an 40 affinity for natural silk with the other dyes.

45 In order further to illustrate my invention, but without being limited thereto, the following specific example is given.

## Example

A velvet having a back of natural silk and a pile of cellulose acetate yarn is treated with a paste consisting of:

|              | Parts by weight |
|--------------|-----------------|
| British gum  | 75              |
| Caustic soda | 150             |
| Water        | 775             |

50 The British gum is boiled with 6 times its 55

weight of water and allowed to cool. The caustic soda is dissolved in the remaining water and allowed to cool. The British gum paste is then added to the caustic soda solution with constant stirring, and the paste strained.

The fabric is treated on a printing machine, the paste being applied on the back of the fabric. After printing the fabric is taken over the back of the printing machine and allowed to dry at room temperatures for 1.5 to 2 hours after which it is rinsed in water, scoured with water containing 5 cc. of hydrochloric acid per litre, then rinsed in water, after which it may be treated in any desired manner.

15. The velvet may be finished with the entire pile erect. However, if it is desired to obtain further differential lustre effects, the velvet may be finished so as to have the cellulose acetate yarn erect and the saponified yarn lying at an angle 20 so as to give a jacquard effect. This may be done by taking the velvet finished by drying with the pile erect and running the same through water and then brushing across the piece of the fabric so as to lay the pile towards the selvage and the pieces then dried. This leaves the saponified 25 cellulose acetate pile lying down flat and the cellulose acetate pile standing practically erect. The fabric is then steamed and cross brushed in opposite direction to make the cellulose acetate pile stand erect without disturbing the position of the laid down saponified pile.

It is to be understood that the foregoing detailed description is given merely by way of illustration and that many variations may be made therein without departing from the spirit 30 of my invention.

Having described my invention, what I desire to secure by Letters Patent is:

1. The method of producing ornamental effects on pile fabrics comprising locally applying to a fabric having a pile comprising organic ester of cellulose yarn a saponifying agent for the organic ester of cellulose and then finishing the fabric by applying pressure to the pile so that the saponified pile yarn occupies a position that is at 40 an angle different from that of the unsaponified organic ester of cellulose pile yarn.

2. The method of producing ornamental effects on pile fabrics comprising locally applying to a fabric having a pile comprising cellulose acetate yarn a saponifying agent for the cellulose acetate and then finishing the fabric by applying pressure to the pile so that the saponified pile yarn occupies a position that is at an angle different from that of the unsaponified cellulose acetate pile yarn.

3. A pile fabric having a differential lustre effect, a part of the pile thereof comprising unsaponified organic ester of cellulose yarn and another part of the pile comprising saponified organic ester of cellulose yarn, the saponified organic ester of cellulose yarn occupying a position that is at a different angle to the face of the fabric than that of the unsaponified organic ester of cellulose yarn.

4. A pile fabric having a differential lustre effect, a part of the pile thereof comprising unsaponified cellulose acetate yarn and another part of the pile comprising saponified cellulose acetate yarn, the saponified cellulose acetate yarn occupying a position that is at a different angle to the face of the fabric than that of the unsaponified cellulose acetate yarn.

5. The method of producing ornamental effects on pile fabrics comprising locally applying to

a fabric having a pile comprising organic ester of cellulose yarn a saponifying agent for the organic ester of cellulose and then finishing the fabric by applying pressure to the pile so that the saponified pile yarn lies flat and the unsaponified pile yarn is substantially erect. 5

6. The method of producing ornamental effects on pile fabrics comprising locally applying to a fabric having a pile comprising cellulose acetate yarn a saponifying agent for the cellulose acetate and then finishing the fabric by applying pressure to the pile so that the saponified pile yarn lies flat and the unsaponified pile yarn is substantially erect.

7. Process for the production of ornamental effects on pile fabrics, which comprises locally applying to a fabric having a pile containing organic ester of cellulose yarn a saponifying agent for the organic ester of cellulose, treating the fabric to cause the pile yarns to assume an 15 erect position and then finishing the fabric by applying pressure to the pile so that the saponified pile yarn occupies a position that is at an angle different from that of the unsaponified pile 20 yarn.

8. Process for the production of ornamental effects on pile fabrics, which comprises locally applying to a fabric having a pile containing cellulose acetate yarn a saponifying agent for the cellulose acetate, treating the fabric to cause the pile 25 yarns to assume an erect position and then finishing the fabric by applying pressure to the pile so that the saponified pile yarn occupies a position that is at an angle different from that of the unsaponified pile 30 yarn.

9. Process for the production of ornamental effects on pile fabrics, which comprises locally applying to a fabric having a pile containing organic ester of cellulose yarn a saponifying agent for the organic ester of cellulose, treating the 40 fabric to cause the pile yarns to assume an erect position and subjecting the fabric to an aqueous treatment and brushing the same so that the saponified pile 45 yarn occupies a position that is at an angle different from that of the unsaponified pile yarn.

10. Process for the production of ornamental effects on pile fabrics, which comprises locally applying to a fabric having a pile containing cellulose acetate yarn a saponifying agent for the cellulose acetate, treating the fabric to cause the pile 50 yarns to assume an erect position and subjecting the fabric to an aqueous treatment and brushing the same so that the saponified pile 55 yarn occupies a position that is at an angle different from that of the unsaponified pile yarn.

11. Process for the production of ornamental effects on pile fabrics, which comprises locally applying to a fabric having a pile containing organic ester of cellulose yarn a saponifying 60 agent for the organic ester of cellulose, treating the fabric to cause the pile yarns to assume an erect position and subjecting the fabric to an aqueous treatment and brushing the same so that the saponified pile 65 yarn lies flat and the unsaponified pile yarn is substantially erect.

12. Process for the production of ornamental effects on pile fabrics, which comprises locally applying to a fabric having a pile containing cellulose acetate yarn a saponifying agent for the cellulose acetate, treating the fabric to cause the pile 70 yarns to assume an erect position and subjecting the fabric to an aqueous treatment and brushing the same so that the saponified 75

pile yarn lies flat and the unsaponified pile yarn is substantially erect.

13. A pile fabric having a differential lustre effect, a part of the pile thereof comprising unsaponified organic ester of cellulose yarn and another part of the pile comprising saponified organic ester of cellulose yarn, the saponified pile yarn lying flat and the unsaponified pile yarn being substantially erect.

14. A pile fabric having a differential lustre effect, a part of the pile thereof comprising unsaponified cellulose acetate yarn and another part of the pile comprising saponified cellulose acetate yarn, the saponified pile yarn lying flat and the unsaponified pile yarn being substantially erect. 5

HERBERT PLATT.